

1

2,901,334

## REMOVAL OF IRON FROM ALUMINUM SURFACES

Melvin H. Brown, Allegheny Township, Westmoreland County, Pa., assignor to Aluminum Company of America, Pittsburgh, Pa., a corporation of Pennsylvania

No Drawing. Application April 9, 1958  
Serial No. 727,272

3 Claims. (Cl. 41—42)

This invention relates to, and has as an object, a convenient, economical treatment for surfaces of aluminum articles to remove iron impurities therefrom. As generally used herein, the term "aluminum" includes both aluminum of various grades and aluminum base alloys.

Containers and other articles made of aluminum and aluminum base alloys are widely used in the chemical industries, and generally may be employed without special surface treatment. However, it has been found that iron impurities on the surfaces of such articles are extremely undesirable for certain applications by reason of the effect which the iron may have upon the material contained or contacted, or even upon the resistance to corrosion of the aluminum article itself. For example, a small amount of iron on the surface of the aluminum sometimes has a contaminating effect in that it is found to promote undesired polymerization of certain plastics or to catalyze the decomposition of hydrogen peroxide.

It has now been found that iron impurities may be removed from the surfaces of aluminum and aluminum base alloy articles by a method in which the article is treated with an aqueous solution containing at least 0.05 percent by weight of soluble citrate ion and at least 0.005 percent by weight of soluble sulfite ion, and having a pH below about 7.0. This method is very effective in removing rolled-in iron, or iron left on an aluminum surface after fabrication.

The ions used in the method just described may be introduced as citric and sulfurous acids, or as soluble salts of these acids, such as sodium, potassium and ammonium citrates and sulfites, bisulfites, or mixtures thereof. Although large concentrations of citrate ion may be employed, it is preferred to use a solution containing less than about 5 percent by weight since amounts in excess of this provide little or no additional benefit and unduly increase the cost of the solution. Similarly, large concentrations of sulfite ion may be employed, but little additional benefit is derived. Generally, a solution containing less than about 10 percent by weight and preferably less than about 5 percent by weight of sulfite ion is utilized. It is desirable that the combined concentration of sulfite and citrate ions total at least 0.1 percent by weight.

The pH of the cleaning solution must be less than 7.0. Generally, the preferred solutions have a pH between 1.0 and 5.0. As is well known, the pH of the solution may be adjusted by introducing the ions as the acids and neutralizing with a base whose salts are soluble, such as ammonium, potassium and sodium hydroxides. To lower the pH, a non-interfering acid such as sulfuric acid may be employed. The more acid solutions, i.e., pH below about 1.0, produce a significant amount of etching which may, however, be disregarded

2

for most applications. It is preferred to use a solution having a pH above about 1.0 to minimize such etching, as well as from the standpoint of handling and disposal.

The surface may be treated with a solution by immersing the entire article in the solution, or by filling the article with the solution, or by running or spraying the solution over the surface, or in any other manner by which the contact may be effected between the solution and the surface. Generally, agitation or movement of the solution relative to the surface of the article shortens the required period of treatment. When the spray method is employed, there is an increased tendency for the sulfite ion to oxidize in contact with air, as well as to decompose and release sulfur dioxide into the air, quite frequently reducing the effectiveness of the solution.

A simple but effective test for the presence of iron impurities on an aluminum surface is the ferroxyl test, wherein the surface is wet with a solution containing 3 percent by weight of potassium ferricyanide and 3 percent by weight of nitric acid. If any iron is present, a blue spot will form within a few seconds. The test solution should be prepared daily since it deteriorates rapidly upon standing. After such a test, the precipitate formed should be removed prior to the treatment of the present invention since it has been found to interfere with the cleaning action. Soap and brushing may be effectively employed to accomplish this removal.

The time of treatment by the method of the invention will vary with the severity of the iron contamination, the composition of the solution and the mode of effecting contact. Treatment times between  $\frac{1}{2}$  and 100 hours are not uncommon; however, treatment times of less than 24 hours are generally sufficient in the treatment of the normally encountered contamination. If the solution is agitated against the surface, treatment times may often be reduced by as much as 40 to 75 percent over those required in an unagitated immersion treatment.

The solutions used in accordance with the present invention are especially adapted for use at room temperature, i.e., ambient temperatures normally prevailing in commercial and industrial atmospheres such as between about 15 and 40° C. However, these solutions may also be employed with lesser effectiveness at elevated temperatures such as 50° C.

Illustrative of the efficacy of the present invention is the following table representing the results obtained in the treatment of prepared test specimens containing embedded iron powder, the contamination being considerably more severe than would be generally encountered. The specimens were immersed in cleaning solutions constituted in accordance with this invention and which were maintained at room temperature unless otherwise noted. Referring to the specimens, one group was an aluminum base alloy nominally composed of aluminum, 3.5 percent magnesium and 0.25 percent chromium (designated in the table as A); a second group was one of the commercial grades of aluminum containing a minimum of 99.60 percent aluminum and a maximum of 0.04 percent manganese (designated as C). The time to cleanance of the impurities generally consisting of silicon and iron (designated as B); the third group was an aluminum base alloy nominally composed of aluminum and 1.2 percent manganese (designated as C). The time to clean reflects the time at which there was no, or an insignificant amount of, iron contamination remaining, as determined by the ferroxyl test.

Table of examples

| Citrate<br>Ion,<br>Percent<br>by wt. | Sulfite<br>Ion,<br>Percent<br>by wt. | pH   | Metal       | Hrs. to<br>Clean | Remarks                                                                           |
|--------------------------------------|--------------------------------------|------|-------------|------------------|-----------------------------------------------------------------------------------|
| 0.05                                 | 0.04                                 | 3.06 | A<br>B<br>C | 48<br>48<br>48   | Added as citric acid and sodium bisulfite.                                        |
| 0.05                                 | 5.0                                  | 2.55 | A<br>B<br>C | 1<br>0.5<br>2    | Added as citric acid and sodium bisulfite. pH adjusted with sulfuric acid.        |
| 5.0                                  | 0.01                                 | 1.8  | A<br>B<br>C | 8<br>8<br>8      | Added as citric acid and sodium sulfite.                                          |
| 5.0                                  | 3.8                                  | 2.55 | A<br>B<br>C | 2<br>0.5<br>2    | Added as citric acid and sodium bisulfite.                                        |
| 1.0                                  | 1.0                                  | 5.0  | A<br>B<br>C | 96<br>48<br>24   | Added as citric acid and sodium bisulfite. pH adjusted with ammonium hydroxide.   |
| 0.8                                  | 3.0                                  | 3.1  | A<br>B<br>C | 48<br>24<br>24   | Added as citric acid and potassium sulfite. pH adjusted with potassium hydroxide. |
| 0.8                                  | 1.5                                  | 3.1  | A<br>B<br>C | 0.5<br>2<br>2    | Added as citric acid and sodium bisulfite. pH adjusted with sodium hydroxide.     |
| 1.7                                  | .19                                  | 1.55 | A<br>B<br>C | 1<br>1<br>1      | Added as citric acid and sodium bisulfite. pH adjusted with sulfuric acid.        |
| 0.8                                  | 1.5                                  | 3.1  | A<br>B<br>C | 0.5<br>2<br>2    | Added as citric acid and sodium bisulfite.                                        |
| 1.34                                 | 0.005                                | 2.18 | A<br>B<br>C | 8<br>2<br>96     | Do.                                                                               |
| 1.8                                  | 0.19                                 | .25  | A<br>B<br>C | 4<br>0.5<br>4    | Added as citric acid and sodium bisulfite. pH adjusted with sulfuric acid.        |
| 0.8                                  | 1.5                                  | 3.1  | A<br>B<br>C | 4<br>4<br>24     | Maintained at 50° C. Added as citric acid and sodium bisulfite.                   |

Of the solutions identified in the foregoing table, it is preferred to employ the solution comprised of 0.8 percent by weight of citrate ion and 1.5 percent by weight of sulfite ion, at room temperature; and this solution may conveniently be made up with citric acid and sodium bisulfites.

Having thus described the invention, I claim:

1. The method of removing iron impurities from a surface of an aluminum article which comprises treating said surface with an aqueous solution consisting essentially of at least 0.05 percent by weight of soluble citrate ion and at least 0.005 percent by weight of soluble sulfite ion, and having a pH below about 7.0.

2. The method in accordance with claim 1 wherein

said solution is at a temperature between about 15 and 40° C.

3. The method of removing iron impurities from a surface of an aluminum article which comprises treating said surface with an aqueous solution consisting essentially of at least 0.05 percent by weight of soluble citrate ion and at least 0.005 percent by weight of soluble sulfite ion, and having a pH of between about 1.0 and 5.0.

#### References Cited in the file of this patent

#### UNITED STATES PATENTS

2,710,792 McDonald ----- June 14, 1955

UNITED STATES PATENT OFFICE  
CERTIFICATE OF CORRECTION

Patent No. 2,901,334

August 25, 1959

Melvin H. Brown

It is hereby certified that error appears in the printed specification of the above numbered patent requiring correction and that the said Letters Patent should read as corrected below.

Column 2, line 64, after "percent" strike out "manganese (designated as C). The time to clean" and insert instead -- copper and 0.01 percent manganese. The bal- --.

Signed and sealed this 9th day of February 1960.

(SEAL)

Attest:

KARL H. AXLINE

Attesting Officer

ROBERT C. WATSON  
Commissioner of Patents